

J. A. BAILEY.

APPARATUS FOR REDUCING THE ORES OF PRECIOUS METALS.

No. 315,886.

Patented Apr. 14, 1885.



Attest:

*Malter Donaldson*  
*J. L. Middleton*

*Inventor*  
*John A. Bailey.*  
*By*  
*Joyce Spear*  
*Attest.*

(No Model.)

2 Sheets—Sheet 2

J. A. BAILEY.

APPARATUS FOR REDUCING THE ORES OF PRECIOUS METALS.

No. 315,886.

Patented Apr. 14, 1885.



Attest:

*W. L. Donaldson*  
*J. L. Middleton*

Inventor:  
John A. Bailey  
by *George A. Pease*  
Attest.

# UNITED STATES PATENT OFFICE.

JOHN A. BAILEY, OF DETROIT, MICHIGAN.

## APPARATUS FOR REDUCING THE ORES OF PRECIOUS METALS.

SPECIFICATION forming part of Letters Patent No. 315,886, dated April 14, 1885.

Application filed August 11, 1884. (No model.)

*To all whom it may concern:*

Be it known that I, JOHN A. BAILEY, of the city of Detroit, county of Wayne, State of Michigan, have invented a new and useful Improvement in Apparatus for Reducing the 5 Ores of the Precious Metals, and I do hereby declare that the following is a full, clear, and exact description of the same.

My invention relates to the reduction of gold, 10 silver, and other ores by means of a crucible or melting-pot, filled with lead or its equivalent, set in a furnace and having suitable appliances for continuously feeding the pulverized and heated mineral onto and through the 15 melted lead, the noble metal in the ore being absorbed by and alloyed with the fused base metal and the refuse mineral cast out.

The apparatus is illustrated in the accompanying drawings, in which similar letters refer to similar parts.

Figure 1 is a central vertical section of one form of my apparatus; Fig. 2, a transverse section on the line 3 4. Fig. 3 is a plan of the cover of the crucible. Fig. 4 is a development 25 of the interior of the crucible on a plane of which the circular line  $x x$  in Fig. 2 is the horizontal trace. Figs. 5 and 6 show another form of my apparatus, the sections being similar to those in Figs. 1 and 2. Fig. 7 is a trans- 30 verse section.

These figures represent a crucible or melting-pot and the mechanism for feeding the pulverized mineral, the furnace by which the whole apparatus is heated, the steam or gas generator, and the method of applying power to rotate the several parts being omitted as not essential to the proper delineation and comprehension of the invention, and to avoid complication in the drawings.

In the figures, A represents a crucible or melting-pot which is filled with lead up to the dotted line. Into the cylinder  $k$  the pulverized mineral is fed through an opening in the top, (not shown in the drawings,) and is kept 40 in motion by the stirrers fixed to the revolving shaft  $o$ , and led to the chute  $j$ , through which it descends into the conveyer-box  $g$  onto the conveyer  $h$ , by which it is carried to the chute  $f$ , which passes through the cover  $e$  of the 45 crucible A, and whence it falls onto the surface 50

of the metal in the crucible A. On each side of the box  $g$  is a large pipe,  $l$ , into which steam can be admitted by the pipe  $n$ , and there superheated and forced into the box  $g$  through the pipe  $m$ .

Referring now to Sheet No. 1, in the center of the crucible A is a tube,  $c$ , which extends nearly to the bottom and passes through the cover  $e$ . This cover  $e$  is made in two parts bolted together, and also bolted to the top of the crucible A, as shown in plan in Fig. 3. Above the cover  $e$  is a guide box and bearing,  $u$ , for the shaft B, having a water-jacket around the shaft at  $w$ . Between this guide-box  $u$  and the top of the tube  $c$  is an insulating-layer of asbestos felt,  $r$ . The shaft B passes down through the center of the tube  $c$  below the surface of the metal, and has attached to its lower end a propeller,  $y$ , which runs freely in the tube  $c$ . Below the propeller  $y$  there is a vertical dia- 65 phragm placed across the tube  $c$ .

At the proper distance above the surface of the metal the nozzles  $d$  are fastened to the tube  $c$ , curving downward and outward, so as to bring their mouths over the center of the vertical tubes  $c'$  and  $c''$ . These tubes have mouth-pieces  $e'$  formed in double cones, and they extend from just below the surface of the metal to a point somewhat above the bottom of the tube  $c$ . On one side of each of them at the bottom 70 are the outlets  $s$ .

Between the central tube,  $c$ , and the inside of the crucible A are the partitions  $f'$ ,  $f''$ ,  $f'''$ , and  $f''''$ . These are best shown in the development of the tubes  $c'$   $c''$  and partitions as 85 given in Fig. 4. Partitions  $f'$  and  $f''$  are attached at their upper ends to the cover  $e$ , and extend nearly to the bottom of the crucible A, and through them pass the bottom openings of the tubes  $c'$  and  $c''$ . Partition  $f''''$  extends to the same depth, but does not rise quite to the surface of the metal, while partition  $f'''$  dips below the top of partition  $f''''$  and rises to the cover  $e$ .

Figs. 5 and 6 show another form in which 95 the feeding mechanism is the same as above described; but in the crucible the tube  $c$  does not rise quite to the surface of the metal, and is surrounded by a larger tube,  $e$ , which replaces the cover  $e$  (shown in Fig. 1) and rises 100

to the plate  $r$ , which is supported above the crucible  $A$  by the brackets  $s'$ . Above this plate  $r$  is an asbestos insulator and guide-box,  $u$ , similar to the one described in Fig. 1. The 5 spout  $f$  from the conveyer-box is attached to the tube  $e$  and delivers the pulverized mineral into it on the surface of the metal. This tube  $e$  at its lower end dips below the surface of the metal, and outside of it is the conical 10 deflecting-tube  $d$ , with its top a little below the top of tube  $c$ . The propeller  $y$  is fastened to the lower end of the shaft  $B$ , and above it are the radial rods  $y'$ , passing through the shaft. Below the propeller  $y$  is the vertical 15 diaphragm  $z$ , placed across the tube  $c$ . At the bottom of the crucible  $A$  is the discharge-pipe  $r'$ , which can be closed by a screw-plug or a clay ball.

When in operation, the whole apparatus is 20 inclosed in a furnace and raised to a heat sufficient to keep the metal in the crucible  $A$  in a fluid condition, and also to raise the mineral in the receiving-cylinder  $k$  to the same or to a higher temperature.

25 The method of operation is as follows: The pulverized mineral is fed into the cylinder  $k$  through an opening in the top, (not shown in the drawings,) and is there heated and kept in motion by the stirrers on the shaft  $o$ , and 30 then passes down the chute  $j$  into the box  $g$ . As it is absolutely necessary to have the air excluded from the fused metal, that it may not be "sickened" or oxidized, steam is admitted through the pipes  $n$  into the pipes  $l$ , where it 35 is superheated and forced through the pipes  $m$  into the box  $g$ , out of which it presses the air up through the falling mineral in the chute  $j$ .

In place of superheated steam, hydrogen 40 gas or hydrocarbon vapor can be introduced under pressure, to force out the air and be mixed with the pulverized mineral. The mineral is then moved forward by the conveyer  $h$  to the chute  $f$ , through which it falls onto the 45 surface of the metal in the crucible  $A$ . Up to this point the action in the two forms shown is the same, but subsequently it is different. Taking, first, the form shown in Figs. 1 and 2, the propeller  $y$  in the tube  $e$  being started, 50 the fluid metal is raised in the tube till it overflows into the nozzles  $d'$ , thence it falls into the conical mouths  $e'$  of the tubes  $c'$  and  $c''$ , creating a downward current in these tubes, which 55 carries with it the pulverized mineral floating on the surface of the metal, and forces it through the bottom openings,  $s$ , whence it rises again to the surface. All the particles of ore are thus brought in contact with the fused metal, and an alloy is formed between it and 60 the precious metal in the ore. If all of this metal is not taken up, it can be passed through a second or a third time, until only refuse mineral rises to the surface. Now, to keep this refuse separate from the metal-bearing ore is the 65 office of the partitions shown. The mineral fed through the chute  $f$  falls between the par-

titions  $f'$  and  $f'''$ , which retain it until it is carried down through the tube  $c$  by the metal current. It then passes out of the opening  $s$  in the bottom of tube  $c$ , and rises on the other side of the partition  $f'$  to the surface, and then the current carries it to and down tube  $c'$ , whence it rises beyond the partition  $f''$ , and is confined between that and partition  $f'''$ . Here there is an opening in the cover  $e$ , (shown in Fig. 3,) out of which the refuse mineral can flow or be removed. Partitions  $f''$  and  $f'''$  are so arranged that the metal can flow back underneath the floating refuse to supply the downward current in the tubes. The cover  $e$  80 being tight, and the partitions  $f'$  and  $f''$  rising up to it, the escape of the steam or gas which enters with the pulverized mineral is prevented, and thus the surface of the fluid metal between these partitions cannot be oxidized, and although there is an opening in the other half of the cover  $e$  for the removal of the refuse very little oxidation can take place on account of the refuse mineral deeply covering the surface. As the propeller  $y$  by its revolutions would create a vortex in the fluid metal, which is very injurious to the proper action of the apparatus, the vertical diaphragm is placed below it across the tube  $c$ , which breaks up the whirling motion. 95

I do not confine myself to the number of tubes and partitions here shown, as in practice there can be one or more, as found necessary for the quality of ore which is to be operated upon.

In the form shown in Figs. 5 and 6 the pulverized mineral falls from the chute  $f$  upon the surface of the metal inside the tube  $e$ . Then, the propeller  $y$  being started in the opposite direction to that used in the other form, 105 a downward current is created in the tube  $c$ , and the mineral is carried down by it, escaping from beneath the tube and rising outside of it to the surface. The radial rods  $y'$ , passing through the shaft  $B$  above the propeller  $y$ , 110 serve to break up any agglomeration of the pulverized mineral which may occur in the upper part of the tube  $c$ . The deflector-tube  $d$  throws the rising refuse outward, where it 115 can be removed, and the arrangement of the ends of the concentric tubes  $d$ ,  $e$ , and  $c$  is such that the fluid metal can return to the tube  $c$  underneath the floating refuse.

To prevent the prejudicial vortex action in the melted metal, the vertical diaphragm  $z$  is 120 placed beneath the propeller  $y$  across the tube  $c$ . After the metal in the crucible has taken up as much of the precious metal as in practice is found best it can be run off through the vent  $r'$  and parted in the usual manner.

Heretofore it has been the general practice 125 to recover the precious metals from their ores by forming an amalgam or alloy with mercury; but there are many ores on which mercury has but little effect, and in all there is a large percentage of loss; but when the assayer desires to ascertain the amount of metal in an ore he 130

does not use mercury, but he melts it with lead and then parts the metals, and thus always obtains a much larger quantity than can be got by the mercury process. The advantage of this apparatus, therefore, is that the assayer's method is practically carried out on a large scale, and thus a much greater proportion of the precious metals can be recovered. This process can also be applied to the reduction of other ores than those containing gold and silver. For instance, copper can be recovered by running the pulverized ore into a bath of melted zinc, which can afterward be distilled off.

15 I am aware that an attempt has been made to pass the ores of the precious metals into a bath of melted lead both by mechanical means and by a vortex created in the lead by a fan-wheel; but

20 What I claim, and desire to secure by Letters Patent, is—

1. In an apparatus for the reduction of ores, the central tube with nozzles and contained propeller so arranged in a crucible containing 25 molten metal as to create an upward current in the tube and through the recurved nozzles, and a downward current in tubes arranged beneath the said nozzles, thereby bringing the pulverized mineral into intimate contact with the molten metal, substantially as described.

30 2. In an apparatus for the reduction of ores, the combination of a central tube having nozzles and a contained propeller with the side

tubes and partitions arranged substantially as described, whereby the continuous supply of 35 pulverized mineral fed into the crucible is carried by the currents created one or more times through the molten metal, the refuse gathering at one side, where it may be removed, substantially as described.

3. In an apparatus for the reduction of ores, the combination of a transverse vertical diaphragm in a central tube containing a propeller with a crucible containing molten metal so arranged that the whirling motion set up by 45 the action of the propeller will be broken and no vortex formed in the fluid metal, substantially as described.

4. The combination of the receiving-cylinder *k*, connected by chute *j* to the conveyer-box 50 *g*, having suitable connections for the admission of steam or gas, and the discharge-chute *f*, with a crucible having a cover and central tube with nozzles containing a propeller and shaft and a transverse diaphragm, together 55 with side tubes and partitions, all contained in a suitable furnace, substantially as described, and for the purposes set forth.

In testimony whereof I have signed my name to this specification in the presence of two sub- 60 scribing witnesses.

JOHN A. BAILEY.

Witnesses:

ALBERT D. PIERCE,  
C. D. FARR.